

## 1

3,629,115

FLUOROSILICONE LUBRICANTS CONTAINING  
TRIS (PENTAFLUOROPHENYL) PHOSPHINE  
Yung Ki Kim and Ogden R. Pierce, Midland, Mich., as  
signors to Dow Corning Corporation, Midland, Mich.  
No Drawing. Filed Aug. 1, 1969, Ser. No. 846,934  
Int. Cl. C10m 1/44, 1/50

U.S. Cl. 252—49.9

2 Claims

## ABSTRACT OF THE DISCLOSURE

Small amounts of tris(pentafluorophenyl)phosphine are added to fluoroalkylpolysiloxane lubricants as antioxidants and anti-wear additives.

This invention relates to improved fluoroalkylpolysiloxane lubricants which contain a minor amount of tris(pentafluorophenyl)phosphine. Addition of the phosphine inhibits oxidation of the fluids and enhances the anti-wear characteristics of metal on metal lubrication.

Organophosphorus compounds are known lubricity additives for organopolysiloxanes in general—see U.S. Pat. 2,684,336. The use of phosphates and phosphites as anti-wear additives in fluorosilicone lubricants is discussed in U.S. Pat. 3,386,917.

By the practice of the present invention, wherein tris(pentafluorophenyl)phosphine is used as an additive, not only are the anti-wear characteristics of fluorosilicone lubricants improved, but the oxidative stability of the fluid is increased, thus preventing the formation of sludge at higher temperatures.

Accordingly, it is an object of the invention to provide an improved fluoroalkylpolysiloxane lubricant.

The invention provides a composition consisting essentially of

(1) 100 parts by weight of an organopolysiloxane fluid containing at least 70 mol percent of



units, any remaining units being of the formula  $(R'\text{SiO}_{3/2})$ ,  $(R'_2\text{SiO})$  or  $(R'_3\text{SiO}_{1/2})$ , in which  $R_1$  is a perfluoroalkyl radical of no more than 12 carbon atoms, R is a lower alkyl radical of no more than 6 carbon atoms or a phenyl radical; R' is a monovalent hydrocarbon or monovalent halohydrocarbon radical; and (2) from 0.1 to 8 parts by weight of tris(pentafluorophenyl)phosphine.

As described above  $R_1$  can be any perfluoroalkyl radical of no more than 12 carbon atoms, for example, heptafluoropropyl, perfluorobutyl, perfluoroisohexyl, prefluorooctyl, perfluorododecyl or, preferably, trifluoromethyl.

R can be the phenyl radical or any of the lower alkyl radicals such as methyl, isopropyl, t-butyl or hexyl. The same or different R substituent can be bonded to the same silicon atom.

R' can be any monovalent hydrocarbon radical, for example, alkyl radicals such as methyl, ethyl, isopropyl, 2-ethylhexyl or octadecyl; aliphatically unsaturated radicals such as vinyl, allyl, ethynyl, butadienyl or 4-hexenyl; or aryl-containing radicals such as phenyl, tolyl, xenyl, naphthyl, benzyl, or 2-phenylpropyl.

R' can also be any monovalent halohydrocarbon radical, for example, 3,3,3-trifluoropropyl, chloropropyl, bromohexyl, chloroallyl, dibromophenyl, chlorophenyl,  $\alpha,\alpha,\alpha$ -trifluorotolyl or chloroxenyl.

## 2

The tris(pentafluorophenyl)phosphine additive is a known compound and can be prepared by the reaction of pentafluorophenyl magnesium bromide and phosphorus trichloride. Only minor amounts, from 0.1 to 8 parts per 100 parts of lubricant, are necessary to obtain the desired oxidative stability. Greater amounts can be used if desired but are generally uneconomical. Depending upon the specific composition of the fluid, insolubility of the phosphine at greater concentrations may present problems.

The following examples are illustrative of the invention which is properly delineated in the claims.

## EXAMPLE 1

15 To determine the efficiency of tris(pentafluorophenyl) phosphine as an anti-oxidant, various amounts of the compound were mixed with portions of trimethylsiloxyendblocked 3,3,3-trifluoropropylmethylpolysiloxane fluid having a viscosity of 300 cs. at 70° F. The oxidative stability of these additive-containing fluids was tested by observing the time required for the fluids to gel at certain high temperatures in open containers. Test conditions and results are given below:

|                               | Weight percent of additive in fluid | Gel time (hrs.) at— |         |         |
|-------------------------------|-------------------------------------|---------------------|---------|---------|
|                               |                                     | 500° F.             | 550° F. | 600° F. |
| One gram in aluminum dish...  | None -----                          | 2                   | 1       |         |
| 30                            | 0.2 -----                           | 4                   | 4       | 4       |
|                               | 1.0 206                             | 123                 |         | 23      |
| Ten grams in 50 ml. beaker... | None -----                          | 15.5                | 6       |         |
|                               | 0.2 23                              | 48                  | 26      |         |
|                               | 1.0 804                             | 206                 |         | 75      |

35 A mixture of 50 grams of the above described fluorosilicone fluid (contain 1 weight percent tris(pentafluorophenyl)phosphine) and 0.5 gram of mineral oil was placed in a 250 milliliter beaker and heated for 2 hours at 550° F. After heating for this period of time, there was no formation of sludge or gummy deposits. This is to be contrasted with testing when an additive-free mixture of the same components is utilized, wherein there is formation of a large amount of sludge. This ability to prevent sludge formation is especially important in those fluids used in hydraulic systems which are highly susceptible to plugging.

## EXAMPLE 2

50 The anti-wear properties of the additive-containing fluorosilicone fluid described above were demonstrated by tests made on the Alpha LFW-1 test machine described in U.S. Pat. 3,028,746. The machine was run in the oscillating mode, using a standard steel ring ( $R_c$  70) and an  $R_c$  30 steel block at a 10° arc and 75 cycles/minute. The 55 wear scar was measured after 5000 cycles and is recorded below:

|    | Weight percent additive in fluid: | Scar dia. (mm.) |
|----|-----------------------------------|-----------------|
| 60 | None -----                        | .90             |
|    | 1% -----                          | .47             |
|    | 5% -----                          | .40             |

65 The additive-containing fluid also gave improved lubrication at high loadings in the four-ball test. With test conditions of 1200 r.p.m. at 167° F. for 30 minutes at a loading of 10 kilograms of steel on aluminum, the addition of 1% tris(pentafluorophenyl)phosphine to the lubricant reduced the scar diameter from 4.9 millimeters to 0.49 millimeter.

**3**  
**EXAMPLE 3**

When from 1 to 7 grams of tris(pentafluorophenyl)phosphine are added to 100 grams of



the oxidative stability of the lubricant is improved.

That which is claimed is:

1. A composition consisting essentially of  
(1) 100 parts by weight of an organopolysiloxane fluid containing at least 70 mol percent of



units, any remaining units being of the formula  $(R'SiO_{3/2})$ ,  $(R'_2SiO)$  or  $(R'_3SiO_{1/2})$ , in which

$R_f$  is a perfluoroalkyl radical of no more than 12 carbon atoms,

R is a lower alkyl radical of no more than 6 carbon atoms or a phenyl radical;

**4**

$R'$  is a monovalent hydrocarbon or monovalent halohydrocarbon radical; and

- (2) from 0.1 to 8 parts by weight of tris(pentafluorophenyl)phosphine.

- 5 2. The composition of claim 1 wherein ingredient (1) is a polymer of 3,3,3-trifluoropropylmethyl siloxane units which have trimethylsiloxy endblocking units.

**References Cited****UNITED STATES PATENTS**

|           |         |               |       |            |
|-----------|---------|---------------|-------|------------|
| 3,078,229 | 2/1963  | Cox           | ----- | 252—49.9 X |
| 3,115,465 | 12/1963 | Orloff et al. | ----- | 252—49.9 X |
| 3,385,790 | 5/1968  | Davies et al. | ----- | 252—52     |
| 3,386,917 | 6/1968  | Schiefer      | ----- | 252—49.9   |
| 3,393,151 | 7/1968  | Dolle et al.  | ----- | 252—49.9   |
| 3,481,872 | 12/1969 | Dolle et al.  | ----- | 252—49.9   |

DANIEL E. WYMAN, Primary Examiner

20 W. H. CANNON, Assistant Examiner

U.S. Cl. X.R.

252—54